

# United States Patent [19]

Mayer et al.

[11] 3,993,852

[45] Nov. 23, 1976

[54] **PROCESS FOR FLAMEPROOFING  
ORGANIC FIBER MATERIALS BY THE  
TRANSFER PROCESS**

[75] Inventors: **Fritz Mayer**, Haltingen, Germany;  
**Jörg Kern**, Oberwil; **Hermann  
Nachbur**, Dornach, both of  
Switzerland

[73] Assignee: **Ciba-Geigy AG**, Basel, Switzerland

[22] Filed: **June 18, 1974**

[21] Appl. No.: **480,339**

[30] **Foreign Application Priority Data**

June 22, 1973 Switzerland..... 9187/73  
July 26, 1973 Switzerland..... 10926/73

[52] **U.S. Cl.**..... **428/921; 8/2.5 A;**  
101/470; 427/248 R

[51] **Int. Cl.<sup>2</sup>**..... **C23C 11/00; C09K 3/28**

[58] **Field of Search**..... 117/136; 252/8.1;  
106/15 FP; 427/390, 394, 248; 8/2.5 A;  
156/230; 101/470; 428/921

[56] **References Cited**

UNITED STATES PATENTS

|           |        |                      |         |
|-----------|--------|----------------------|---------|
| 3,559,317 | 2/1971 | Knight et al. ....   | 117/3.2 |
| 3,645,936 | 2/1972 | Gardner.....         | 117/136 |
| 3,650,820 | 3/1972 | DiPietro et al. .... | 117/136 |
| 3,660,582 | 5/1972 | DiPietro et al. .... | 117/136 |

|           |         |                     |         |
|-----------|---------|---------------------|---------|
| 3,666,402 | 5/1972  | Meyers et al. ....  | 117/136 |
| 3,707,346 | 12/1972 | Markert et al. .... | 8/2.5   |
| 3,715,310 | 2/1973  | Butcher .....       | 117/136 |
| 3,915,628 | 10/1975 | Bossard et al. .... | 8/2.5   |

**FOREIGN PATENTS OR APPLICATIONS**

1,243,219 8/1971 United Kingdom

*Primary Examiner*—Michael R. Lusignan  
*Attorney, Agent, or Firm*—Joseph G. Kolodny; Edward  
McC. Roberts; Prabodh I. Almaula

[57] **ABSTRACT**

New phosphorus compounds are provided which correspond to the formula



wherein R<sub>1</sub> and R<sub>2</sub> each denote alkyl with 1 to 6 carbon atoms, X denotes alkylene with 1 to 4 carbon atoms and A denotes phenyl substituted by hydroxyl, alkoxy with 1 to 4 carbon atoms, alkoxy carbonyl with 2 to 5 carbon atoms, phenyl or halogen and n is 1 or 2. These compounds are useful as flameproofing agents for organic fiber material, especially for polyamide, polyacrylonitrile or linear polyester fibers, when applied according to the dry thermal transfer process.

**11 Claims, No Drawings**

**PROCESS FOR FLAMEPROOFING ORGANIC FIBER MATERIALS BY THE TRANSFER PROCESS**

The subject of the invention is a process for flameproofing organic fibre material by the dry thermal transfer process, characterised in that a preparation which contains at least

a. a phosphorus compound of the formula



10

(1)

wherein  $R_1$  and  $R_2$  denote alkyl with 1 to 6 carbon atoms,  $X$  denotes alkylene with 1 to 4 carbon atoms and  $A$  denotes phenyl, or phenyl substituted by hydroxyl, alkoxy with 1 to 4 carbon atoms, alkyl with 1 to 4 carbon atoms, alkoxy carbonyl with 2 to 5 carbon atoms, phenyl or halogen, and  $n$  is 1 or 2,

b. optionally a binder which is stable below 250° C and

c. optionally a solvent is applied to an inert carrier and is optionally dried, the carrier is then brought into contact with the surface of the fibre material which is to be flameproofed, thereafter the carrier and the material to be finished are subjected to a heat treatment at not less than 80° C, if appropriate with use of mechanical pressure, until the phosphorus compound has been transferred to the fibre material, and the finished material is then separated from the carrier.

Particularly suitable phosphorus compounds are those of the formula



(2)

wherein  $A_1$  denotes phenyl or phenyl substituted by hydroxyl or alkoxy carbonyl with 2 to 5 carbon atoms and  $R_1$ ,  $X$  and  $n$  have the indicated meaning.

Phosphorus compounds particularly suitable for the process according to the invention are those of the formula



(3)

wherein  $A_2$  denotes phenyl, hydroxyphenyl, alkoxy carbonylhydroxyphenyl or hydroxydiphenyl and  $R_1$  and  $n$  have the indicated meaning.

Advantageous results are obtained above all with phosphorus compounds of the formula



(4)

wherein  $R_3$  denotes methyl or ethyl,  $n$  denotes 1 or 2 and  $A_3$  denotes phenyl, 3-methoxycarbonyl-4-hydroxyphenyl or 3-phenyl-4-hydroxyphenyl.

Compounds of the formula (1) which are suitable above all are, for example, the following phosphorus compounds:



(5)

wherein  $R_1$  and  $R_2$  each denote alkyl with 1 to 6 carbon atoms,  $X$  denotes alkylene with 1 to 4 carbon atoms and  $A_4$  denotes phenyl substituted by hydroxyl, alkoxy with 1 to 4 carbon atoms, alkyl with 1 to 4 carbon atoms, alkoxy carbonyl with 2 to 5 carbon atoms, phenyl or halogen, and  $n$  is 1 or 2.

Particularly suitable phosphorus compounds are those of the formula



(6)

wherein  $A_5$  denotes phenyl substituted by hydroxyl or alkoxy carbonyl with 1 to 5 carbon atoms and  $R_1$ ,  $X$  and  $n$  have the indicated meaning.

Phosphorus compounds which are in particular suitable for the process according to the invention are those of the formula



(7)

wherein  $A_6$  denotes hydroxyphenyl, alkoxy carbonyl-hydroxyphenyl or hydroxydiphenyl and  $R_1$  and  $n$  have the indicated meaning.

Advantageous results are achieved above all with phosphorus compounds of the formula



(8)

wherein  $R_3$  denotes methyl or ethyl,  $n$  denotes 1 or 2 and  $A_7$  denotes 3-methoxycarbonyl-4-hydroxyphenyl or 3-phenyl-4-hydroxyphenyl.

Examples of suitable compounds of the formula (1) are the following phosphorus compounds:



(9.1)



(9.2)

(9.3)



(9.4)



(9.5)



(9.6)



(9.7)



(9.8)



Amongst these, the compound of the formula (9.2) is particularly preferred.

R<sub>1</sub> and R<sub>2</sub> in the formulae (1), (2), (3), (5), (6) and (7) preferably represent alkyl with 1 to 4 carbon atoms. For example, R<sub>1</sub> and R<sub>2</sub> each denote n-hexyl, n-butyl, tert. butyl, isopropyl, n-propyl and especially 55 ethyl or methyl.

A is phenyl or, in particular, a substituted phenyl radical. For example, A represents toluyl, phenyl or, above all, 4-hydroxyphenyl, 3-methoxycarbonylphenyl, 3-phenyl-4-hydroxy-phenyl, cresyl, chlorophenyl or 60 bromophenyl or, in particular, 3-methoxycarbonyl-4-hydroxy-phenyl.

X preferably represents methylene, but radicals such as ethylene, n-propylene or n-butylene are also possible.

The compounds of the formulae (1) and (2) are known or are manufactured according to methods which are in themselves known, for example by reac-

tion of the corresponding benzoic acid ester with a corresponding phosphite.

In particular, the compounds which are unsubstituted in the phenyl nucleus are known, whilst the compounds which are substituted in the phenyl nucleus are new but can be manufactured according to known methods.

Accordingly, a further subject of the invention are the new phosphorus compounds of the formulae (5), (6), (7), (8) and especially (9.2).

10 A further subject of the invention relates to a process for the manufacture of phosphorus compounds of the formula (5), characterised in that a compound of the formula



20 wherein X denotes alkylene with 1 to 4 carbon atoms, Y denotes halogen, Z<sub>1</sub> and Z<sub>2</sub> each denote alkoxy with 1 to 4 carbon atoms, alkyl with 1 to 4 carbon atoms, 25 alkoxy carbonyl with 1 to 5 carbon atoms, phenyl, halogen or an optionally acylated hydroxyl group with 2 to 5 carbon atoms in the acyl radical, and m and n are 1 or 2, is reacted with a phosphite of the formula



35 wherein R<sub>1</sub>, R<sub>2</sub> and R<sub>4</sub> each denote alkyl with 1 to 6 carbon atoms, in the melt at 100° to 180° C, and, if n is 1, a divalent nickel halide is co-used as the catalyst, and, if relevant, the acylated hydroxyl groups of the 40 phosphorus compound obtained are subsequently hydrolysed.

To manufacture the phosphorus compounds of the formula (6), compounds of the formula



are employed, wherein Z<sub>3</sub> and Z<sub>4</sub> each denote alkoxy-carbonyl with 2 to 5 carbon atoms or an optionally acylated hydroxyl group with 2 to 5 carbon atoms in the acyl radical and X, Y, m and n have the indicated meaning.

To manufacture the phosphorus compounds of the formula (7), compounds of the formula



are employed, wherein Y denotes halogen, m and n each denote 1 or 2, Z<sub>6</sub> denotes alkoxy carbonyl with 2

to 5 carbon atoms or phenyl and, if  $Z_6$  is alkoxy carbonyl and  $m$  is 2,  $Z_5$  denotes a free hydroxyl group, or, if  $Z_6$  is phenyl and  $m$  is 2 or if  $m$  is 1,  $Z_5$  denotes an acylated hydroxyl group with 2 to 5 carbon atoms in the acyl radical.

To manufacture the phosphorus compounds of the formula (8) compounds of the formula



are employed, wherein  $Y_1$  is chlorine or bromine,  $n$  is 1 or 2,  $Z_8$  is phenyl or methoxycarbonyl and, if  $Z_8$  is methoxycarbonyl,  $Z_7$  is hydroxyl or, if  $Z_8$  is phenyl,  $Z_7$  denotes acetyl.

5-Bromo-2-hydroxy-benzoic acid methyl ester is employed for the manufacture of the compound of the formula (9.2).

To manufacture the compounds of the formulae (6) and (7), phosphites of the formulae



are employed, wherein  $R_1$  denotes alkyl with 1 to 6 carbon atoms.

To manufacture the compounds of the formula (8), phosphites of the formula



are employed, wherein  $R_3$  denotes methyl or ethyl.

To manufacture the compound of the formula (9.2), triethyl phosphite is employed.

The reaction is preferably carried out at 140°-190° C, especially at 170° to 180° C, the corresponding alkyl halide  $R_1Y$  or  $R_2Y$ , especially methyl bromide or ethyl bromide or methyl chloride or ethyl chloride, being split off.

The divalent nickel halide which is optionally co-used in the reaction if  $n$  in the formula (10) is 1, is nickel-(II) bromide or especially nickel-(II) chloride.

If  $Z_1$ ,  $Z_2$ ,  $Z_3$ ,  $Z_4$  and  $Z_5$  in the formulae (10), (12) and (13) denote an acylated hydroxyl group, and especially if  $Z_7$  in the formula (14) denotes an acetyl group, the reaction gives acylated, especially acetylated, phosphorus compounds, of which the acylated, especially acetylated, hydroxyl group is hydrolysed to the free hydroxyl group.

This hydrolysis is suitably carried out in a solvent or in a solvent mixture in which the phosphorus compound obtained is soluble, under alkaline ammoniacal conditions, at the boiling point of the solvent or solvent mixture used.

The solvents or solvent mixtures employed are, for example, alkanols with 1 to 4 carbon atoms, such as methanol and especially ethanol, and/or, for example,

aliphatic saturated monoketones with 3 to 6 carbon atoms, such as 2-hexanone, methyl propyl ketone, acetone or especially methyl ethyl ketone. Ethanol, or a mixture of ethanol and methyl ethyl ketone in the ratio of 1:1 are particularly suitable.

The hydrolysis is carried out in an alkaline ammoniacal medium, preferably employing aliphatic amines with 1 to 4 carbon atoms, preferably dialkylamines or trialkylamines, or mixtures of these amines, especially diethylamine.

During the hydrolysis, the corresponding aliphatic, saturated monocarboxylic acids with 2 to 5 carbon atoms, especially acetic acid, are split off.

The preparations which can be used in accordance with the process can contain, in addition to the phosphorus compound of the formula (I), at least one binder which is stable below 250° C, water and/or an organic solvent.

Suitable binders are synthetic, semi-synthetic and natural resins, and in particular both polycondensation and polyaddition products. In principle, all binders customary in the lacquer and printing ink industry can be used. The binders serve to retain the phosphorus compounds of the formula (1) on the treated position of the carrier. At the transfer temperature they should, however, not melt, not react with themselves, for example crosslink, and be capable of releasing the compound to be transferred. Preferred binders are those which, for example, dry rapidly in a warm stream of air

20 and form a fine, preferably non-tacky, film on the carrier. As examples of suitable water-soluble binders there may be mentioned: alginate, tragacanth, carubin (from carob bean flour), dextrin, etherified or esterified vegetable mucins, carboxymethylcellulose or polyacrylamide, whilst as binders soluble in organic solvents there may be mentioned cellulose esters, such as nitrocellulose or cellulose acetate and especially cellulose ethers, such as methylcellulose, ethylcellulose, propylcellulose, isopropylcellulose, benzylcellulose or

25 hydroxyethylcellulose as well as their mixtures. Particularly good results are achieved with ethylcellulose. As organic solvents it is possible to use water-miscible or water-immiscible organic solvents or solvent mixtures of boiling point below 150° C, preferably 30 below 120° C, under normal pressure. Advantageously, aliphatic, cycloaliphatic or aromatic hydrocarbons, such as toluene, cyclohexane, or petroleum ether, lower alkanols, such as methanol, ethanol, propanol, isopropanol, esters of aliphatic monocarboxylic acids, 35 such as ethyl acetate or propyl acetate, aliphatic ketones, such as methyl ethyl ketone and halogenated aliphatic hydrocarbons, such as perchloroethylene, trichloroethylene, 1,1,1-trichloroethane or 1,1,2-trichloro-2,2,1-trifluoroethylene are used. Particularly 40 preferred solvents are lower aliphatic esters, ketones or alcohols, such as butyl acetate, acetone, methyl ethyl ketone, ethanol, isopropanol or butanol, as well as their mixtures, for example a mixture of methyl ethyl ketone and ethanol in the ratio of 1:1. The desired viscosity of

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 90

aration. The amounts of compound, to be transferred to the fibre material, applied to the temporary carrier can be, for example, 10 to 100 g, preferably 15 to 40 g, per m<sup>2</sup> of carrier.

The preparations which can be used according to the invention are prepared by dissolving or finely dispersing the phosphorus compound of the formula (1) in water and/or organic solvent, advantageously in the presence of a binder which is stable below 250° C.

Further, it is also possible, and also particularly advantageous, to apply compounds of the formula (1) direct as such onto the carrier, that is to say without adding solvent or binder, for example by spraying, doctoring, pouring or sprinkling.

The process according to the invention is suitably carried out by applying the preparations to an inert temporary carrier, bringing the treated side of the carrier into contact with the fibre material which is to be treated, subjecting the carrier and the fibre material to the action of heat at not less than 80° C, preferably not less than 130° C, and separating the fibre material from the carrier.

The temporary carrier required in accordance with the process can be endless or be matched to the textile shapes which are to be treated, that is to say cut into shorter or longer pieces. As a rule it has no affinity for the preparation used. Suitably, the carrier is a flexible, preferably dimensionally stable, band, a strip or a film, preferably having a smooth surface, which is stable to heat and can consist of materials of the most diverse kind, for example metal, such as an aluminum foil or steel foil, plastic, paper or textile sheet-like structures, such as woven fabrics, knitted fabrics or fleeces which can optionally be coated with a film of vinyl resin, ethylcellulose, polyurethane resin or polytetrafluoroethylene.

Suitably, flexible aluminum foils, sheets of glass fibre fabric or above all sheets of paper are used.

After the preparations have been applied to the carrier, they are dried, for example by means of a warm stream of air or by infra-red irradiation, the solvent used optionally being recovered.

The treated side of the carrier is thereupon brought into close contact with the surface to be dyed of the fibre material, and the combination is subjected to a heat treatment at not less than 80° C and preferably 150° to 220° C, particularly 150° to 200° C.

These temperatures are maintained for a sufficient period of time, preferably 5 to 120 seconds, until the flameproofing agent has been transferred to the fibre material to be treated.

Changes in temperature and in time can result in corresponding changes in the amount of coating for the same chemicals presented. It is therefore possible to regulate the transfer of the chemicals to the fibre material, and hence the amount of coating, through regulating the temperature and the transfer time.

The exposure to heat can be effected in various known ways, for example by means of a heating plate or by passing through a tunnel-shaped heating zone or over a hot heating drum, advantageously in the presence of an unheated or heated counter-roller which exerts pressure, or through a hot calendar, or by means of a heated plate (iron or warm press), optionally in vacuo, the heating devices being preheated to the requisite temperature by steam, oil or infra-red radiation or being located in a preheated chamber. After com-

pletion of the heat treatment, the textile goods are separated from the carrier.

Preferably, in addition to natural fibre materials such as cellulose, synthetic fibre materials are treated in accordance with the invention, such as, for example, cellulose ester fibre, such as cellulose 2½-acetate and triacetate fibres, especially synthetic polyamide fibres, for example those from poly-ε-caprolactam (nylon 6), from polyhexamethylenediamine adipate (nylon 6,6) or from poly-ω-aminoundecanoic acid (nylon 7), polyurethane or polyolefine fibers, for example polypropylene fibres, acid-modified polyamides, such as polycondensation products of 4,4'-diamino-2,2'-diphenyldisulphonic acid or 4,4'-diamino-2,2'-diphenylalkanedisulphonic acids with polyamide-forming starting materials, polycondensation products of monoaminocarboxylic acids or their amide-forming derivatives or of di-basic carboxylic acids and diamines with aromatic dicarboxysulphonic acids, for example polycondensation products of ε-caprolactam or hexamethylenediammonium adipate with potassium 3,5-dicarboxybenzenesulphonate, or acid-modified polyester fibres, such as polycondensation products of aromatic polycarboxylic acids, for example terephthalic acid or isophthalic acid, polyhydric alcohols, for example ethylene glycol and 1,2- or 1,3-dihydroxy-3-(3-sodium sulphopropoxy)-propane, 2,3-dimethylol-1-(3-sodium-sulphopropoxy)-butane, 2,2-bis-(3-sodium-sulphopropoxyphenyl)-propane or 3,5-dicarboxybenzene sulphonic acid or sulphonated terephthalic acid, sulphonated 4-methoxybenzenecarboxylic acid or sulphonated diphenyl-4,4'-dicarboxylic acid.

Preferably, however, fibre material of polyacrylonitrile or acrylonitrile copolymers and above all linear polyester fibres, especially of polyethylene glycol terephthalate or poly-(1,4-cyclohexanedimethyol) terephthalate, are used. If acrylonitrile copolymers are used, the proportion of acrylonitrile is suitably at least 50% and preferably at least 85 per cent by weight of the copolymer. The comonomers used are normally other vinyl compounds, for example vinylidene chloride, vinylidene cyanide, vinyl chloride, methacrylates, methylvinylpyridine, N-vinylpyrrolidone, vinyl acetate, vinyl alcohol, acrylamide or styrenesulphonic acids.

These fibre materials can also be used as mixed fabrics, the fibre materials being mixed with one another or with other fibres, examples being mixtures of polyacrylonitrile/polyester, polyamide/polyester, polyester/viscose and polyester/wool.

The fibre material can be in the most diverse states of processing, for example in the form of flocks, tow, yarn, texturised filaments, woven fabrics, knitted fabrics, fibre fleeces or textile floor coverings, such as especially needle-punched felt carpets, pile carpets or bundles of yarn.

The preparations which can be used according to the invention are applied to the temporary carrier by, for example, whole-area or partial spraying, coating or printing.

The temporary carriers can also be treated on both sides or, if appropriate, on the back, and unequal concentrations of the coatings can be selected for the two sides.

In the manufacturing instructions and examples which follow, percentages are percentages by weight.

## MANUFACTURING INSTRUCTIONS

## A. Compound of the formula (9.2)

23.1 g of 5-bromo-2-hydroxy-benzoic acid methyl ester and 0.5 g of nickel-(II) chloride are heated to 170° C, while stirring. 16.6 g of triethyl phosphite are then added dropwise at this temperature. The solution first turns deep blue-violet and then the reaction commences, with vigorous foaming, the ethyl bromide formed being evolved. The reaction is complete with no further ethyl bromide escapes. 15.1 g of the compound of the formula (9.2), which distils at boiling point 0.01 mm Hg = 129 to 131° C, are obtained.



Analysis: Calculated : C 50.0%, H 5.94%, P 10.73%.  
Found : C 49.88%, H 5.87%, P 10.55%.

## B. Compound of the formula (9.3)

20.1 g of 5-chloromethyl-2-hydroxy-benzoic acid methyl ester are heated as a melt to 100° C and 16.6 g of triethyl phosphite are slowly added at this temperature over the course of 50 minutes; towards the end of the dropwise addition an exothermic reaction, with a temperature rise of about 10° C, can be observed, which ceases after addition of the triethyl phosphite. The reaction mixture is subsequently further heated to 140° C and is kept at this temperature for 1 hour, during which the initially colourless reaction mixture assumes a slight yellowish discolouration. 25.0 g of the compound of the formula (9.3) are obtained.



Analysis: Calculated : C 51.66%, H 6.25%, P 10.58%.  
Found : C 51.62%, H 6.34%, P 10.25%.

## C. Compound of the formula (9.4)

50.15 g of 5-chloromethyl-2-hydroxy-benzoic acid methyl ester are heated as a melt to 100° C, and 31 g of trimethyl phosphite are added sufficiently slowly that the temperature does not rise above 110° C. After addition of the trimethyl phosphite, the reaction mixture is further heated to 160° C and is kept at this temperature for 1 hour. The compound of the formula (9.4) is distilled as a crude product at 0.01 mm Hg, only the fraction distilling at 147° C being collected, as a slightly turbid oil of refractive index  $n_{20}^{\circ}$  1.5292.



Analysis: Calculated : C 48.18%, H 5.51%, P 11.30%.  
Found : C 47.88%, H 5.44%, P 11.12%.

## D. Compound of the formula (9.5)

29.1 g of 2-acetyl-5-bromo-diphenyl and 0.5 g of nickel-(II) chloride are heated to 170° C, whilst stirring. 16.6 g of triethyl phosphite are added to this suspension at 170° C over the course of 1 hour. The reaction commences, with vigorous foaming, immediately after the start of the addition of the triethyl phosphite and the reaction mixture assumes a blue-violet colour. The addition of triethyl phosphite is regulated in such a way that the ethyl bromide formed by the reaction distils off without delay. After the addition, the reaction mixture is kept at 170° C for approx. 30 minutes, until no further ethyl bromide distils.

The reaction product is then purified by vacuum distillation. 21.8 g of 2-acetyl-diphenyl-5-phosphonic acid diethyl ester are obtained in the form of a clear, colourless, oil distillate (boiling point 122°–126° C at 0.08 mm Hg).

2-Acetyl-diphenyl-5-phosphonic acid diethyl ester, thus obtained, 7.7 g of diethylamine and 4.5 g of ethanol are kept at the reflux temperature for 1 hour. Thereafter the by-products (triethylamine and acetic acid) are removed from the dark brown, oily reaction mixture by distillation at 0.05 mm Hg. The yellow crystalline distillation residue is twice recrystallised from carbon tetrachloride. 12.1 g of the compound of the formula (9.5) are obtained as white, crystalline needles. Melting point 156° C.



Analysis: Calculated : C 62.74%, H 6.25%, P 10.22%.  
Found: C 61.9%, H 6.3%, P 10.3%.

## E. Compound of the formula (9.6)

50.0 g of 3-ethyl-benzyl chloride are heated to 120° C and 53.7 g of triethyl phosphite are added over the course of 2 hours, in the course of which gaseous ethyl chloride formed by the reaction is evolved. After completion of the addition of triethyl phosphite, the reaction mixture is further heated to the reflux temperature of 140° C and kept under reflux for 15 hours. The crude product is then purified by vacuum distillation. 56.2 g of the compound of the formula (9.6) are obtained as distillate. (Boiling point 120° C at 0.1 mm Hg).



Analysis: Calculated: C 60.92%, H 8.30%, P 12.08%.  
Found: C 61.17%, H 8.37%, P 12.00%.

## F. Compound of the formula (9.7)

54 g of 3-methoxy-benzyl chloride are heated to 120° C and 57.3 g of triethyl phosphite are added over the course of 45 minutes, during which time gaseous ethyl chloride formed by the reaction is evolved. After completion of the addition of triethyl phosphite, the reaction mixture is further heated to 190° C. Thereafter, 5 g of unreacted triethyl phosphite are removed from the reaction mixture at 22° C and 0.1 mm Hg. 76 g of the compound of the formula (9.7) are obtained as a distillation residue, which is in the form of a pale yellowish liquid.



Analysis: Calculated: C 55.81%, H 7.42%, P 11.99%.  
Found : C 56.78%, H 7.32%, P 11.12%.

## G. Compound of the formula (9.8)

97.9 g of 3-chloro-benzyl chloride are heated to 120° C and 100.1 g of triethyl phosphite are added at this temperature over the course of 45 minutes, during which time gaseous ethyl chloride formed by the reaction is evolved. After the addition, the reaction mixture is kept for 15 hours at the reflux temperature, the latter rising gradually from 130° to 170° C. Unreacted triethyl phosphite is then removed from the reaction mixture at 25° to 50° C and 0.04 mm Hg. 111 g of the compound of the formula (9.8) are obtained as a distillation residue, which is in the form of a clear liquid.



Analysis: Calculated: C 50.30%, H 6.14%, Cl, 13.50%, P 11.79%.  
Found : C 49.35%, H 6.06%, Cl, 14.66%, P 11.24%.

## EXAMPLE 1

12 g of the compound of the formula (9.2) are applied to a paper carrier of 1 m<sup>2</sup> surface area.

The carrier is placed with the coated side downwards on top of a polyester woven fabric (120 g/m<sup>2</sup>). The

## 11

carrier and the fabric are packaged in an aluminium foil and exposed to a heat treatment at 195°C for 25 seconds. The carrier and the fabric are then separated from one another. The polyester fabric proves to have a flameproof finish according to DIN 53,906 (ignition time 3 seconds), in contrast to the untreated fabric. The tear length is 7 cm and the burning time is 4 seconds. The untreated test specimen burns away.

Similar results are also obtained when using one of the compounds of the formulae (9.1), (9.3), (9.4) or (9.5).

## EXAMPLE 2

The phosphorus compound of the formula (9.2) is applied by doctor blade or spraying into a glass fibre fabric (coating 30 g/m<sup>2</sup>). The glass fibre fabric is brought together with a polyamide woven fabric, with the coated side facing away from the latter. The carrier and the fabric are then subjected to a heat treatment at 195°C between two heated plates for 30 seconds. The glass fibre fabric is then separated from the polyamide fabric without objectionable adhesion of the layer of chemicals to the finished polyamide fabric.

The polyamide fabric is found to be flameproofed according to DIN 53,906 (ignition time 3 seconds), in contrast to the untreated fabric.

## EXAMPLE 3

750 g of the product of the formula (9.2) are worked into a paste in 100 g of ethylcellulose and 350 g of a 1:1 mixture of ethanol and methyl ethyl ketone, and applied to paper at the rate of 24 or 48 g/m<sup>2</sup>.

The coated side of the carrier is brought into contact with a polyester knitted fabric (240 g/m<sup>2</sup>) and the combination is subjected to a heat treatment at 195°C between two heating plates for 25 seconds. The carrier and the knitted fabric are then separated from one another.

The knitted fabrics are then tested for their flame resistance according to DOC FF 3-71 ("Children's Sleepwear Test"), the test being carried out after the finishing process and also after 1, 5, 10, 20 and 40 use-type washes at 40°C in a liquor containing 4 g/l of a commercial detergent for delicate fabrics.

The result is summarised in Table 1 which follows.

Table 1

|                                      | Coating, g/m <sup>2</sup> | Finishing |    | 1 wash |    | 5 washes |    | Tested after |    | 40 washes  |    |
|--------------------------------------|---------------------------|-----------|----|--------|----|----------|----|--------------|----|------------|----|
|                                      |                           | TL        | BT | TL     | BT | TL       | BT | TL           | BT | TL         | BT |
| Untreated                            |                           | 12        | 22 | 4      | 9  | 10       | 25 | 4            | 19 | Burns away |    |
| Treated with compound of the formula |                           |           |    |        |    |          |    |              |    |            |    |
| (9.2)                                | 24                        | 5         | 2  | 7      | 2  | 6        | 2  | 5            | 1  | 5          | 1  |
| (9.2)                                | 48                        | 5         | 0  | 7      | 1  | 4        | 2  | 5            | 1  | 5          | 1  |

TL : Tear length in cm

BT : Burning time in seconds

DOC FF 3-7 ("Children's Sleepwear Test") is the following flameproofing test:

5 Pieces of fabric (8.9 cm x 25.4 cm) are clamped in a test frame and dried for 30 minutes at 105°C in a circulating air drying cabinet. The pieces of fabric are subsequently conditioned in a closed vessel over silica gel for 30 minutes and then subjected to the actual flame-resistance test in a burning box. The fabrics are in each case ignited for 3 seconds with a methane gas flame, the fabrics being in the vertical position.

## 12

The test is considered to have been withheld if the average charred zone is not longer than 17.5 cm and no one sample has a charred zone of more than 25.4 cm, and the individual smouldering times are not longer than 10 seconds.

## EXAMPLE 4

10 g of one of the compounds of the formulae (9.1), (9.4), (9.6), (9.7) or (9.8) are applied by doctor blade to an aluminium foil (coating: 60 g/m<sup>2</sup>).

The aluminium foil is placed on a polyacrylonitrile fibre carpet (pile weight 600 g/m<sup>2</sup>), the coated side of the foil being brought into contact with the carpet pile. The carpet backing and the uncoated side of the foil are subjected to the action of heat at 200°C between two heated plates for 30 seconds.

The carpet treated in this way and an untreated carpet are tested for their flame resistance according to DIN 51,960, the results being summarised in Table 2 below:

Table 2

| Carpet treated with compound of the formula | Diameter of the burning zone in cm | Burning time in minutes |
|---------------------------------------------|------------------------------------|-------------------------|
| (9.1)                                       | 6.5                                | 3                       |
| (9.4)                                       | 5                                  | 3                       |
| (9.6)                                       | 5                                  | 3                       |
| (9.7)                                       | 5                                  | 3                       |
| (9.8)                                       | 5                                  | 3                       |
| Untreated carpet                            | Burns away completely              | 6                       |

## EXAMPLE 5

Instead of a polyester woven fabric, a polyamide woven fabric (240 g/m<sup>2</sup>) is finished with one of the compounds of the formulae (9.3), (9.7) or (9.8) in the manner indicated in Example 1. The results of the DIN 53,906 test (ignition time 3 seconds) are summarised in Table 3 below.

Table 3

| Polyamide fabric finished with compound of the formula | Burning time in seconds | Tear length in cm |
|--------------------------------------------------------|-------------------------|-------------------|
| (9.3)                                                  | 12                      | 7                 |
| (9.7)                                                  | 8                       | 10                |

|                                 | (9.8) |    |                       |
|---------------------------------|-------|----|-----------------------|
| Polyamide fabric without finish |       | 5  | 7                     |
|                                 |       | 23 | Burns away completely |

We claim:

1. Process for flameproofing organic fiber material by the dry thermal transfer process which comprises applying to an inert carrier a preparation containing a phosphorus compound of the formula



wherein R<sub>1</sub> and R<sub>2</sub> each are alkyl with 1 to 6 carbon atoms, X is alkylene with 1 to 4 carbon atoms and A is phenyl, or phenyl substituted by hydroxyl, alkoxy with 1 to 4 carbon atoms, alkyl with 1 to 4 carbon atoms, alkoxy carbonyl with 2 to 5 carbon atoms, phenyl or halogen, and n is 1 or 2, then bringing the carrier into contact with the surface of the fiber material which is to be flameproofed, thereafter subjecting the carrier and the material to be finished to a heat treatment at 150° to 220° C until the phosphorus compound has been transferred to the fiber material, and then separating the finished material from the carrier.

2. Process according to claim 1 which comprises applying a preparation containing a phosphorus compound of the formula



wherein A<sub>2</sub> is phenyl, hydroxyphenyl, alkoxy carbonyl-hydroxyphenyl or hydroxydiphenyl and R<sub>1</sub> and n have the meaning indicated in claim 1.

3. Process according to claim 2, which comprises applying a preparation containing a phosphorus compound of the formula



wherein R<sub>3</sub> is methyl or ethyl, n is 1 or 2 and A<sub>3</sub> is phenyl, 3-methoxycarbonyl-4-hydroxyphenyl or 3-phenyl-4-hydroxyphenyl.

4. Process according to claim 1, which comprises applying a preparation containing a phosphorus compound of the formula



wherein R<sub>1</sub> and R<sub>2</sub> each are alkyl with 1 to 6 carbon atoms, X is alkylene with 1 to 4 carbon atoms and A<sub>4</sub> is phenyl substituted by hydroxyl, alkoxy with 1 to 4 car-

bon atoms, alkyl with 1 to 4 carbon atoms, alkoxy carbonyl with 2 to 5 carbon atoms, phenyl or halogen, and n is 1 or 2.

5. Process according to claim 4, which comprises applying a preparation containing a phosphorus compound of the formula



wherein A<sub>5</sub> is phenyl substituted by hydroxyl or alkoxy carbonyl with 1 to 5 carbon atoms and R<sub>1</sub>, X and n have the meaning indicated in claim 4.

6. Process according to claim 5 which comprises applying a preparation containing a phosphorus compound of the formula



wherein R<sub>3</sub> is methyl or ethyl, n is 1 or 2 and A<sub>7</sub> is 3-methoxycarbonyl-4-hydroxyphenyl or 3-phenyl-4-hydroxyphenyl.

7. Process according to claim 6 which comprises applying a preparation containing the phosphorus compound of the formula



8. Process according to claim 7 which comprises applying a preparation containing, in addition to the phosphorus compound, a binder which is stable below 250° C and an organic solvent.

9. Process according to claim 1 which comprises applying a preparation containing from 20 to 100 per cent by weight of phosphorus compound 0 to 30 per cent by weight of a binder which is stable below 250° C and 0 to 70 per cent by weight of an organic solvent.

10. Process according to claim 1 which comprises flameproofing polyamide fibers, polyacrylonitrile fibers or linear polyester fibers.

11. The organic fiber material bearing thereon a flameproofing finish applied according to the process of claim 1.

\* \* \* \* \*